

# UNITED STATES PATENT OFFICE.

SAMUEL CABOT, OF BOSTON, MASSACHUSETTS.

## PROTECTIVE SHEETING AND METHOD OF MANUFACTURING THE SAME.

No. 804,376.

Specification of Letters Patent.

Patented Nov. 14, 1905.

Application filed June 23, 1905. Serial No. 266,680.

*To all whom it may concern:*

Be it known that I, SAMUEL CABOT, a citizen of the United States, and a resident of Boston, in the county of Suffolk and State of 5 Massachusetts, have invented new and useful Improvements in Protective Sheeting and Method of Manufacturing the Same, of which the following is a specification.

My invention relates to the preparation and 10 construction of protective sheets; and it consists of an improved method by which the same are prepared and in the finished article of manufacture resulting from the said method. In the manufacture of this sheeting I employ 15 an adhesive composition which consists of paste or paint composed of comminuted solid inorganic incombustible material, preferably a fibrous inorganic material, such as asbestos or asbestiform talc in suspension in an adhesive, which is preferably an inorganic and anti-septic adhesive, such as a solution of borate, boric acid, or silicate of soda or potash, to which mixture may be added, if desired, a pigment to color the coating. The character of the 20 inorganic adhesive mentioned is such that when a coating whereof they constitute a component is set or dried it assumes a hard and brittle condition, so that the continuity of such a coating if laid upon a flexible material 25 or surface will become cracked, broken, and partially detached, and therefore seriously impaired in its resistant and protective qualities. In the preparation of protective sheets, which may be applied as floor or wall coverings or as wrappings for valuable and perishable goods, unless such sheetings be specially contrived and constructed, so that the tendency of the coating to crack off may be successfully obviated, one of the principal pur- 30 poses of the said composition or of compositions analogous thereto, which possess similar physical characteristics, is frustrated. By my improved method of compounding and constructing the protective coating and sheets 35 coated therewith this difficulty is overcome and the manufacture, use, and shipment of such sheets is made readily possible without danger of impairing the continuity of the protective film by the ordinary conditions of 40 use and wear.

The method of preparation of the sheetings is as follows: I take a fibrous sheet of ordinary material—such as cloth, felt, or paper—which when unprotected is combustible and 45 susceptible also to the attacks of the slower oxidation of decay and to the depredations of

insects, and apply to this fibrous and destructible organic sheet a coating of resistant or refractory material such as above described. By reason of the character and consistency of 50 the adhesive employed as the vehicle for the inorganic refractory material the coating is in whole or in part superficial upon the fibrous sheet and in proportion to the weight and thickness of the coating it is brittle and liable 55 to crack irregularly and become locally detached from the sheet after it is hard. Therefore, preferably, while the coated sheets of fibrous material are still soft and the coating itself but recently set I corrugate the sheets. 60 This corrugation may be effected most readily by passing the sheets between corrugated rolls. These corrugations may be straight ridges or wrinkles across the width of the material, and in this condition will enable the 65 material to be rolled quite tightly upon an axis parallel to the corrugations. By this method a resistant inorganic adhesive veneer is applied to a fibrous organic sheet whereof the inherent qualities of strength and flexibility 70 are preserved, while the article of manufacture as an integer is highly refractory and resis- 75 tant to destructive agencies.

The effect of the corrugation of the compound sheet, which consists of the fibrous 80 base and a veneer of protective material, is to seam the veneer or coating with a multitude of minute fissures or cracks, so that the veneer becomes, as it were, a firmly-adhering mosaic composed of very minute and closely-fitting 85 pieces. The advantages of this cracking are that the sheet as a whole may readily be rolled without breaking the substantial continuity of the hard coating, and, further, that under conditions of rapid oxidation, espe- 90 cially on the application of great heat, which generates gases in the body of the fibrous sheet, a great number of microscopic vents are provided, the gases escaping readily through the fissures of the coating. This prevents the 95 accumulation of gas-pressure, which in the case of a continuous and unbroken protective coating, is liable to burst the coating and de- 100 stroy its protective capacity.

In the manufacture of protective sheetings 105 according to this method the proportions of ingredients used in compounding the coating may be varied to suit varying conditions. I have found, however, that for heavy felting a coating compounded as follows is suitable 110 and effective: ten parts, by weight, of borate, boric acid, or silicate of potash or soda dis-

solved in twenty parts, by weight, of water, thirty parts, by weight, of comminuted asbestos or asbestiform talc, and, if desired, a pigment which preferably should not exceed 5 five parts, by weight, of the mixture. For thin felts or paper or for cloth I have found it advisable to modify the composition as follows: using ten parts, by weight, of borate, biborate, or silicate of potash or soda dissolved in ten parts, by weight, of water, ten parts, by weight, of comminuted asbestos or asbestiform talc, and pigment which preferably should not exceed five parts, by weight, in the mixture. Practical demonstration 10 leads me to believe that a coating composed of solid comminuted inorganic refractory material and an adhesive vehicle which is also inorganic and preferably antiseptic constitutes a coating more effective to resist oxidation 15 and other destructive agencies than such inorganic adhesives as the silicates, borates, &c., when applied alone, although these have been found, as is well known, to lend resistant properties to otherwise destructible materials; but whether the adhesive film has incorporated with it or not the comminuted inorganic material, it is, if heavy enough to be an effective protective coating, so brittle 20 when dry and hard that unless suitable measures are contrived to prevent, it will break, crack irregularly, and become locally detached if the material to which it is applied is bent or folded.

My invention, therefore, is applicable to 35 and embraces situations wherein flexible sheets are rendered resistant or refractory by any of the protective coatings which when dry and hard become brittle.

I claim—

40 1. The method of manufacturing protective material which consists in coating a sheet of fibrous organic material with a superficial veneer of inorganic adhesive material, brittle when dry, then drying and corrugating the 45 sheet.

2. The method of manufacturing protective material which consists in coating a sheet of fibrous organic material with a superficial

veneer composed of inorganic comminuted refractory material in suspension in an adhesive vehicle, brittle when dry, then drying and corrugating the sheet. 50

3. The method of manufacturing protective material which consists in coating a sheet of fibrous organic material with a superficial veneer composed of comminuted asbestos in suspension in an inorganic antiseptic adhesive and corrugating the sheet after the coating has set. 55

4. The method of manufacturing protective material which consists in coating a sheet of fibrous organic material with a superficial adhesive inorganic veneer, and subsequently producing a multitude of minute fissures in the veneer. 60

5. The method of manufacturing protective material which consists in coating a sheet of fibrous organic material with an adhesive superficial veneer composed of comminuted inorganic refractory material in suspension 70 in an adhesive, and subsequently producing a multitude of minute fissures in the veneer.

6. A protective sheet composed of fibrous material coated with a superficial veneer of adhesive refractory material, said veneer subdivided by a multitude of minute fissures. 75

7. A protective sheet composed of fibrous organic material, coated with a superficial veneer composed of comminuted inorganic refractory material in suspension in an inorganic adhesive, the veneer subdivided by a multitude of minute fissures. 80

8. A protective sheet composed of fibrous organic material superficially coated with a veneer composed of fibrous inorganic refractory material such as asbestos or asbestiform talc, incorporated with an inorganic adhesive such as borate, biborate or silicate of potash or soda, the said veneer subdivided by a multitude of fissures. 85

Signed by me at Boston, Massachusetts, this 8th day of June, 1905.

SAM. CABOT.

Witnesses:

JOSEPH T. BRENNAN,  
GRACE E. GIBBONS.